

## 1

3,394,090  
METHOD OF FOAMING POLYVINYL CHLORIDE  
USING AN ACTIVATOR

Dieter H. A. Hayer, Stuttgart, Germany, assignor to  
G. Siegle & Co. GmbH, Stuttgart, Germany  
No Drawing. Filed May 11, 1964, Ser. No. 366,654  
1 Claim. (Cl. 260—2.5)

For pressureless production of foam products on the basis of high polymers, especially of polyvinyl chloride and its mixed-polymerizates, there are employed propellants, as, for example, azodicarbonamide and benzene-sulphonehydrazide. In order to be able to carry out this process also at lower temperature it is customary to add to these propellant-added mixtures also an activator or so-called "kicker." For obtaining a sufficient light- and heat-stabilization there is also added to these mixtures a commercial stabilizer.

As activators for polyvinyl chloride and similar high polymers there are usually employed basic lead salts, as, for example, lead carbonate, lead sulphate, lead phthalate, and similar compounds, but also zinc compounds, as, for example, zinc oxide, all of which give a comparatively good kicker-effect. But the heat- and light-stabilization obtained with these products is insufficient for the majority of employment purposes. Moreover, the hitherto-employed products, because of the comparatively great covering ability, exhibit white-pigment characteristics, so that with the employment of such activators it is usually only in special cases that it is possible to obtain dark and deep colortones.

It has now been found that by the employment of salts of bivalent metals and monocarboxylic acids there is obtained not only an excellent kicker effect but at the same time also a very good heat- and light-stabilization. The acids employed are preferably aliphatic aromatic and mixed aliphatic-aromatic monocarboxylic acids with a C-number of 6-14.

Good results are obtained with alpha-phenylbutyric acid, p-tolylic acid, p-chlorobenzoic acid and trichlorobenzylic acid. There are preferably employed aromatic carboxylic acids which contain one or more alkyl- or aryl-groups as well as halogen-groups. As metals there find employment preferably cadmium and lead.

The advantages of the method of the invention can be seen from the following table, in which there is presented the activating and stabilizing effect of the products of the invention in comparison with a commercial activator and a commercial stabilizer at a foaming carried out at 160° C. and a furnace test carried out at 180° C. As the commercial activator there was employed zinc oxide, and as the commercial stabilizer, Nuostabe V-979. The numerical values give the foaming duration in seconds respectively the duration of the heat treatment until a clearly beginning discoloration in minutes.

## 2

|                                            | Foaming Duration in Seconds | Beginning of Discoloration After Minutes |
|--------------------------------------------|-----------------------------|------------------------------------------|
| Commercial activator                       | 160                         | 10                                       |
| Commercial stabilizer                      | 950                         | 45                                       |
| Cadmium salt of alphaphenylbutyric acid    | 158                         | 40                                       |
| Cadmium salt of methylbenzoic acid         | 214                         | 45                                       |
| Lead salt of methylbenzoic acid            | 165                         | 45                                       |
| Cadmium salt of trichlorophenylacetic acid | 229                         | 35                                       |
| Cadmium salt of alpha-ethylhexanoic acid   | 200                         | 45                                       |

The foaming duration was determined in the following manner: 15 grams of diethylphthalate, 15 grams of azodicarbonamide, and 10 grams of a kicker of the invention were maintained in an oil bath at a temperature of 160° C. At this there split off gases, which were captured and measured. After the times stated in the above table the gas evolution was ended. At the furnace test carried out for determining the heat stability the following recipe was employed: 70 parts of polyvinyl chloride (produced according to the suspension method), 30 parts of diethylphthalate, 1 part of lubricant (commercial monooleate), and 1 part of product according to the invention.

The quantity of the activator according to the invention added to the aforementioned substances may be between 0.5 and 10% of the total quantity of the polymer.

A foam product produced according to the invention at low temperature without pressure exhibits the following composition: 100 parts of polyvinyl chloride or polyvinyl chloride-mixed polymerizates; 60 parts of softener, for example, diethylphthalate; 4 parts of propellant, for example, azodicarbonamide; 1 part of a product according to the invention.

What is claimed is:

1. In a method of preparing foam articles from a mixture comprising (a) polyvinylchloride, and (b) a heat decomposable propellant therefor containing a nitrogen-to-nitrogen bond wherein the mixture is heated to an elevated temperature at which the propellant releases gas and the polyvinylchloride is foamed thereby, the improvement which comprises simultaneously activating the propellant and stabilizing the polyvinylchloride by admixing 0.5-10 parts by weight of an activator with each 100 parts by weight of the polyvinylchloride prior to the foaming thereof, the activator consisting of at least one salt of a divalent metal and a monocarboxylic acid containing one aryl group selected from the group consisting of the lead and cadmium salts of alpha phenylbutyric acid, methylbenzoic acid, trichlorophenylacetic acid, p-chlorobenzoic acid and mixtures thereof.

## References Cited

## UNITED STATES PATENTS

- 55 3,197,423 7/1965 Ackerman 260—2.5  
MURRAY TILLMAN, Primary Examiner.  
M. FOELAK, Assistant Examiner.